

May 7, 1935.

H. C. PORTER

2,000,610

PACKAGE BINDER

Filed July 11, 1932

Fig. 2.



Fig. 4.



Fig. 3.



Fig. 5.



Fig. 6.



Fig. 7.



Fig. 1

## UNITED STATES PATENT OFFICE

2,000,610

## PACKAGE BINDER

Howard C. Porter, La Grange Park, Ill., assignor  
to Signode Steel Strapping Company, Chicago,  
Ill., a corporation of Delaware

Application July 11, 1932, Serial No. 621,844

10 Claims. (Cl. 24—20)

My invention relates to package-binders,—particularly such as are used for binding individual packages or for binding groups of packages into assembled units for handling and shipment.

Usually such binders are looped and tightly tensioned around the package or group of packages and then overlapping portions are jointed or sealed together to make the encircling loop permanent. Ordinarily the tension is applied to a portion or reach of an encircling binder at one side of the package or group of packages and consequently, in order effectively to distribute the locally applied tension throughout the encircling binder, it is very desirable that the friction between the binder and the package or group of packages, particularly at the corners, be as low as possible. Otherwise the sections or reaches of binder other than that to which the tension is initially applied may be relatively free from tension and loose so that when the package or group of packages is subsequently subjected to shocks and jars the tension, which theretofore has been to a considerable extent localized, becomes distributed. And then, since some portions were initially relatively loose, the entire binder may be insufficiently tight. Furthermore it is desirable that under some conditions the friction between superposed contacting portions of the binder be as low as possible, particularly when the stretching or tensioning tools employed perform their work by sliding portions of the binder upon and past one another such, for example, as the tools set forth in Flora Patent No. 1,149,569 or in Gunther Patent No. 1,453,564. On the other hand in order to produce a strong and reliable union or joint between the overlapping binder portions—particularly folded or crimped joints of the type set forth in Flora Patent No. 1,252,680 or Leslie Patent No. 1,445,330—it is very desirable that the friction between contiguous overlapping strap portions which are tightly folded or crimped together be as high as possible in order to oppose the tendency of the overlapped and folded portions to separate longitudinally under the tension to which the binder may be subjected.

One of the objects of my invention is to provide a binder wherein normally the coefficient of surface friction is low so that it will readily slide over the surfaces and corners of packages or groups of packages and over portions of like binders, but which when subjected to the bending and pressure incident to the production of a crimped joint, will exhibit a high coefficient of

surface friction to oppose the rupture of the joint.

Another object is to provide a composite coating for a binder, the normal and initially exposed surface having a low coefficient of friction whereas the contiguous surfaces which become exposed in the folded or crimped joint have a high coefficient of friction.

Another object is to provide a double coating for a metallic binder, the outer layer having a low coefficient of friction and the inner layer a high coefficient of friction.

Another object is to provide an attractive, weatherproof and durable finish for metallic package binder,—a finish which in addition to these properties, will facilitate its proper application to packages.

Another object is to provide a process for providing a metallic binder with dual friction surfaces.

Other objects and advantages will hereinafter appear.

In the drawing

Fig. 1 is a perspective of a portion of binder, in the form of a flat strap, with its several surface forming coatings cut back and partly removed,—the constituent parts being very much enlarged and exaggerated in order to illustrate generally their relationship.

Fig. 2 is a top plan of a typical joint, of the folded or crimped type, for uniting contiguous overlapping portions of binder.

Fig. 3 is a side elevation of such a joint,

Fig. 4 is a cross section on the line 4—4 of Fig. 3,

Fig. 5 is a highly magnified cross section through a small portion of binder showing the normal relationship between the core and the high and low friction surfaces,

Fig. 6 is a similar view showing the relationship between the constituent parts of contiguous contacting binder portions when subjected to relatively slight pressure and bending such as obtains during tensioning operations, and

Fig. 7 is a similar view showing the relationship between the parts when the contiguous contacting portions are subjected to the relatively severe pressure and crimping which obtain upon the formation of the joint.

In general my invention contemplates the provision of a metallic package binder such as a steel strap or wire having an inner and normally unexposed surface characterized by a relatively high coefficient of friction and having an outer normally exposed surface characterized

5 by a relatively low coefficient of friction, the surfaces being of such a character that the friction between the binder and packages and between superposed contacting portions of the binder is relatively low during the above mentioned sliding, stretching and tensioning operations, but the friction between contacting binder portions becomes relatively great or high when such binder portions are deformed to produce a 10 union or folded joint of the general type disclosed in the previously mentioned Flora and Leslie patents.

15 The binder illustrated in the drawing has a core 1 consisting of a flexible steel strap or ribbon. The primary or inner normally unexposed surface may take the form of a coating or layer 2 of hard, tough, weatherproof varnish or enamel-like material which will tenaciously 20 adhere to the steel strap or core 1.

25 I do not wish, however, to limit my invention to any particular primary coating, it being essential only that the inner or normally unexposed surface of the strap or core be readily flexible and sufficiently elastic to enable it to bend with the core without flaking off and without crushing, be harder than the outer or secondary relatively smooth surface and provide or maintain a microscopic roughness, such as is 30 commonly known as an eggshell or satin finish, when subjected to joint forming pressure and deformation.

35 The outer or secondary surface is illustrated as a layer or coating 3, which preferably is relatively thin compared to the thickness of the inner or primary coating. This layer or coating may be composed of a semi-hard wax like material having a surface which is dry and relatively very slippery. It should be stable under ordinary temperature conditions so that it will 40 normally remain as a thin covering over the primary surface. But when superposed or overlapping portions of the binder are deformed to produce a folded or crimped joint of the type heretofore mentioned, the primary surface is 45 exposed to permit intimate engagement, within the joint, of the relatively rough high friction surfaces of parts of the overlapping binder portions.

50 I do not know the precise reason or reasons why the outer low friction surface offers low resistance to slipping or relative movement during the tensioning or stretching operation, and yet is so disposed during the bending and clamping operation of joint formation as to expose the surface having a high coefficient of friction. I have observed, however, that when the superposed portions are deformed to produce a 55 folded joint or union, the character of the surfaces in the regions of greatest deformation undergoes a physical change and takes on a minutely flaky or crystalline appearance.

60 It may be that the minute recesses or fissures interspersed among the microscopic flakes or crystals increase the capacity of the primary surface for the reception of the secondary coating or wax-like material so that as the binder is deformed and the fissures form, the secondary coating is ruptured and drawn down into the fissures with the result that the high friction surfaces become exposed and engage each other. On the other hand, it may be that the microscopically rough primary surface sufficiently 65 supports the secondary coating under the pressures incident to tensioning to keep itself covered with the wax-like low friction material,

5 although, when subjected to pressures incident to joint formation, the secondary coating flows into the microscopic recesses of or is pierced by the microscopic projections of the rough primary surface with the result that the projections of the primary surfaces of superposed binder portions become engaged producing high friction.

10 It is, of course, possible that the advantageous results obtained from my invention in actual practice may be due to a combination of the effects of deformation and pressure as above described. But whatever the cause may be, I have observed that while the undeformed binder is smooth, of a satiny or eggshell finish appearance and possesses a low coefficient of surface friction, the deformed binder, particularly along the lines of fold, exhibits the flaky or crystalline appearance and has a relatively high coefficient 15 of surface friction.

20 Microscopic examination of contiguous contacting surfaces seems clearly to indicate that, under relatively slight pressure and bending such as obtains around package corners and in ordinary tensioning tools of the character hereinbefore mentioned, such surfaces are related as illustrated in Fig. 6 wherein the outer secondary coating 3 of wax like low friction material covers and is supported by the minute projections and bridges the minute depressions in the 25 primary high friction surface 2. Thus under such conditions the friction between the contacting surfaces of binder is relatively low. But when the pressure and crimping action is concentrated and severe, as obtains in the folded 30 joint, then the outer coating 3 is pierced by the projections of the high friction inner surface 2 as shown in Fig. 7 and the engagement of these 35 projections results in high friction between the contacting binder surfaces.

40 The primary or inner high friction surface 2 may be provided by a coating composed of various ingredients which will give the desired results. One specific compound may be made by thoroughly mixing 78 pounds of black baking 45 varnish of 10 gallons oil length, 12 pounds of sesqui-oxide of iron pigment finely ground and 10 pounds of light naphtha. This mixture may be applied to the steel strap by spraying, dipping or wiping, as desired, and is then set or 50 hardened by drying, baking for about one hour at approximately 400° Fahrenheit affording good results. The primary or inner surface thus produced is microscopically rough with minute 55 depressions and projections which, under a microscope of about one hundred power, appear to be rather uniformly distributed and of approximately equal area,—the separation of projections being of the order of about .0002 to .001 inch.

60 After the strap is thus covered with the primary coat the secondary or outer coating or surface 3 is applied. Various wax like substances, which are stable at ordinary temperatures, may be applied. A suitable substance may be provided by mixing 12 pounds of petroleum wax of 65 130° Fahrenheit melting point, 50 pounds of carnauba wax, 38 pounds of beeswax and 50 gallons of a suitable thinner, such as turpentine. This mixture may be applied over the primary 70 coat by dipping, spraying or wiping, as desired. After being thus applied it is allowed to dry and, preferably, polished in any suitable manner, such as by being rubbed with or passed between dry felt pads. This secondary coat should be 75

applied very thinly over the primary surface so as to form a smooth slippery surface over the satiny or eggshell finish of the latter.

The binder thus treated has a relatively smooth slippery outer or normally exposed surface 3 which allows one portion to slide freely upon another portion, as in a stretching tool of the type mentioned in the Flora and Guenther patents supra, and to slide freely upon the surface and about the corners of a package or group of packages under such tension as is ordinarily applied for banding or binding purposes. However, when two contiguous overlapping portions of the binder are in a static condition folded and squeezed or crimped together tightly enough to form a joint such as set forth in the Flora and Leslie patents, supra, the minute projections or relatively rough surfaces of the primary coat 2 are exposed and engage each other with great surface friction therebetween. The coatings form a protective covering for the steel core, preventing it from rusting, and, because the outer coat 2 is exceedingly thin and sufficiently transparent to permit the primary coat 2 to show through, the binder has an eggshell or satiny dark reddish brown and attractive appearance. Of course, if other colors are desired they may be obtained by, for example, substituting some other suitable solid pigment. Thus a velvety black may be obtained by the use of graphite.

Having thus described the nature and a specific illustrative embodiment of my invention, what I claim and desire to secure by United States Letters Patent is as follows:

1. A package-binder adapted to be tensioned about packages and made into a permanently closed loop thereabout by a folded joint between overlapping portions, comprising a flexible metallic core having a surface of high coefficient of friction, and a coating of relatively low coefficient of friction which is normally over said surface but disposable to expose said surface of high coefficient of friction in the folded joint.

2. A package-binder adapted to be tensioned about packages and made into a permanently closed loop thereabout by a folded joint between overlapping portions, comprising a flexible metallic core, a primary coating of flexible hard material adhering to the core and having a surface of high coefficient of friction, and a secondary coating of low coefficient of friction normally covering the primary coating but exposing the same when the binder is folded into a joint.

3. A package-binder comprising a flexible metallic core, a primary coating of flexible hard enamel-like material adhering to the core and having a microscopically rough outer surface, and a thin wax like smooth secondary coating over the primary coating, the secondary coating being disposable to expose the rough primary coating when the binder is folded into a joint.

4. A package-binder comprising a flexible metallic core, a primary coating adhering to and covering the core, said primary coating being hard and flexible and with a microscopically rough eggshell finish surface, and a wax like secondary coating over the primary coating, the secondary coating being relatively thin and smooth and disposable when the binder is folded into a joint to expose the primary coating and thereby increase the friction coefficient of 10 the binder.

5. A package-binder comprising a flexible metallic core, a primary coating adhering to and covering the core, said primary coating being hard and having a microscopically rough surface with substantially uniformly distributed depressions and projections of about equal areas, and a wax like secondary coating over the primary coating, the secondary coating being relatively thin and smooth.

6. A package-binder comprising a flexible metallic core, a primary high friction surface coating adhering to and covering the core, said primary coating comprising a hard enamel-like substance including minute particles of a solid 25 metalloid substance, and a wax like secondary coating over the primary coating, the secondary coating being relatively thin and with low friction surface.

7. The method of finishing a metallic package-binder which comprises, giving the binder a primary surface of microscopic roughness with substantially uniformly distributed depressions and projections of about equal area, and covering the primary surface with a coating of 30 thin smooth wax like material which is stable at ordinary temperatures.

8. The method of finishing a metallic package-binder which comprises, applying thereto a primary coating of a liquid enamel-like substance which possesses a high coefficient of friction when set, drying the primary coating to set the same upon the binder into a hard eggshell-finish surface therefor, and applying over the primary coating a thin wax like smooth secondary coating.

9. The method of finishing a metallic package-binder which comprises covering the binder with a primary coating of liquid enamel-like material which dries into a hard coat with microscopically rough high friction surface, drying the primary coating to set the same upon the binder, applying a secondary coating of wax like material over the primary coating, and polishing the secondary coating.

10. The method of finishing a flexible metallic package-binder which comprises applying a primary coating of a varnish-like material containing a finely ground pigment, drying the primary coating to harden the same, and applying over the primary coating a thin smooth 60 secondary coating of wax like material.

HOWARD C. PORTER.